

Sept. 29, 1936.

P. M. J. BARDOU-JOB ET AL

2,055,691

INSULATING MATERIAL FOR LINING AND OTHER USES

Filed April 6, 1934



## UNITED STATES PATENT OFFICE

2,055,691

INSULATING MATERIAL FOR LINING AND  
OTHER USES

Pierre Michel Justin Bardou-Job and Henri  
Francis Hébrard, Perpignan, France, assignors  
to Rè, Saint-Marguerite, Ceret, Pyrenees-  
Orientales, France, a joint-stock company of  
France

Application April 6, 1934, Serial No. 719,258  
In France June 9, 1933

4 Claims. (Cl. 106—23)

Our invention relates to the manufacture of insulating material adapted to be used for lining and other uses.

The object of this invention is in particular 5 to manufacture an insulating material which is very homogeneous and has a very high insulating capacity.

The invention consists primarily in an insulating material characterized by the mixture of 10 cork and sulphur.

In one embodiment of the invention, the sulphur is applied in the state of flowers of sulphur or finely pulverized sulphur.

The insulating material described above 15 comprises two materials only, cork and sulphur. Other materials may however be added to these substances without on that account going outside the scope of the invention.

For example, a certain quantity of ammonium 20 salts or ammonium and magnesium salts may be added. This addition has the advantage of making the insulating material fire resisting.

Colouring matters may also be added to the 25 mixture, such as ochres and sienna earths whereby insulating materials of different colours can be obtained.

When it is desired to improve the qualities 30 of the insulating material, such as the flexibility and firmness, solid or liquid products are added to the mixture, e. g. rubber, boiled or raw linseed oil, latex, etc.; the insulating material obtained is then easy of application on account of its flexibility.

The insulating material according to this 35 invention further comprises the characteristic features which will appear from the following description and more particularly from the appended claims.

The preferred forms of the apparatus for the 40 manufacture of the insulating material according to the present invention are illustrated in the accompanying drawing in which Figures 1 and 2 are two axial sections of two pieces of apparatus according to the invention.

The insulating material according to this 45 invention is composed essentially of a mixture of fragments of cork and sulphur, the latter being advantageously applied in the state of flowers of sulphur or finely pulverized sulphur.

In order to obtain such an insulating material, 50 the cork granules are placed in a container 1 (Figure 1) heated externally by means of steam for example. In order to obtain as rapidly as possible a temperature which is uniformly distributed throughout the mass of granules, the

container 1 is provided with a rotary agitator 2 actuated by a drive 3.

When the maximum temperature comprised 5 between 110° and 120° C. has been reached, the sulphur in the form of flowers of sulphur or powdered sulphur is sprayed upon the granules while continuing to agitate the mass. In this way, the particles of sulphur melt in contact with the granules of hot cork and thus adhere 10 to these granules.

The damper 4 which closes the base of the container 1 is then opened in order to allow the mixture to flow into a mould 5. This discharging operation should be effected as rapidly as possible so that the mixture will not have time to 15 cool. Immediately after the mixture has been run out, it is placed under a press the applied pressure varying according to the purpose of the material to be obtained.

The material is removed from the mould a few 20 minutes later when the temperature has fallen a few degrees. This process has the advantage that it only requires a fairly low temperature (110° to 120° C.). It is therefore very economical and the saving is increased on account of 25 the fact that the temperature is applied to the materials during a short time only.

The invention includes the insulating material 30 thus obtained whatever be the proportion of cork and sulphur, but it also includes a particularly 30 advantageous insulating material containing the following proportion of sulphur and cork:

| By weight |   |     |
|-----------|---|-----|
| Cork      | — | 4/5 |
| Sulphur   | — | 1/5 |

This insulating material has numerous advantages.

In the first place its colour closely resembles 40 that of natural cork and this is due to the low temperature required by the process and further by the relatively low proportion of sulphur, which material has a light colour approaching that of cork. This colour may also when required be modified by the addition of colouring 45 materials as mentioned above.

The insulating material is completely insoluble in water.

As it is formed of two highly insulating materials, the insulating material is a perfect insulator. It can thus be used advantageously as internal linings for modern houses, for which purpose it is still more suitable on account of the fact that it is sound absorbing in addition to being insulating.

A further very interesting advantage of this insulating material resides in the fact that it is not attacked by parasites, such as vegetable parasites. It will be understood that under these 5 conditions this insulating material can be of great service in industry and particularly in modern constructions, for the insulation of refrigerators, for conduits, etc.

Finally, this insulating material has a low 10 specific gravity and on this account imposes only a very small load on constructions on which it is employed.

Numerous modifications may be made in the 15 above described process for the manufacture of the insulating material without on that account going outside the scope of the invention.

Thus, instead of the flowers of sulphur being sprayed upon the previously heated cork granules, the latter may be coated in the cold state 20 with the flowers of sulphur and the mixture thus obtained in the cold state may then be subjected to the action of heat. This operation may be carried out in a similar apparatus to that described above, but nevertheless this mode of 25 procedure gives slightly less satisfactory results than that previously described, because it is fairly difficult to obtain a homogeneous mixture in the cold state.

The insulating material may also be obtained 30 by the immersing and mixing of the cork granules in a mass of molten sulphur or inversely and this operation may be effected, like the foregoing, in the apparatus described above.

The insulating material according to this invention 35 may also be obtained by proceeding in the following manner with the aid of the device illustrated in Figure 2.

The cork granules are placed in the container 1, these granules being previously mixed with the 40 flowers of sulphur. A current of steam is then supplied to this mixture through a pipe 6 which dips into the mixture.

In this way a certain quantity of water is incorporated in the mixture, thereby facilitating 45 the coating of the cork granules with sulphur in the cold state.

The operation is continued as described above by the container 1 being heated externally and by the mixture being agitated by means of the 50 agitator 2.

When the operation has been completed, the mixture is run off as described above by the opening of the damper 4 and this mixture is collected in a mould 5, the discharging operation 55 being effected as rapidly as possible.

It is to be noted that the steam supplied into the mixture at the commencement of the operation commences to heat the mass so that the mixture is already at a certain temperature when 60 heat is applied to the container 1. The supplementary operation which consists in moistening the mixture has therefore no substantial effect upon the total duration of the operation.

There is also a saving in time because this 65 moistening facilitates coating the cork granules with sulphur while the mixture is still cold.

It is also observed that the supply of steam to the mixture heats the mass directly while the

external heating of the container 1 produces an indirect heating of the mass.

The mixture may be moistened by any means other than by the supply of steam to this mixture. For example water may be incorporated 5 directly in the mass in a liquid form. In this case the moistening may be effected in a completely cold state without any addition of heat.

It has been specified above that the mixture of cork and sulphur was heated before moulding. According to one of the features of the present invention the heat may be supplied to the mixture at the moment of moulding. In this case the granules of cork are coated with sulphur in the cold state, the mass is moistened, if necessary, and the mixture is then introduced into the mould. The mixture is then subjected to a certain pressure and is then heated to a temperature comprised between 110° and 120° C. The particles of sulphur melt under the action of the heat and ad- 20 here to the cork granules.

This mode of operation has the following advantage:

The pressure is applied to the mixture at the moment when the temperature corresponds to a 25 maximum viscosity of the sulphur. In this way, the sulphur fills the voids between the cork granules in the most complete possible manner so that a material is finally obtained which is very homogeneous and very compact.

Finally, according to the invention, an insulating material is obtained which possesses the following properties:—

1. Excellent insulation against cold.
2. Excellent insulation against heat.
3. A better electrical installation than other insulating material.
4. Effective resistance to parasites and gnawing on account of the presence of the sulphur.
5. Sanitary materials which are freed from infinitely small germs by the liberation of sulphur dioxide during the heat treatment.
6. Very low inflammability.
7. Very good cohesion.

What we claim is:—

1. Insulating material for linings and other uses, comprising granulated cork, a binder consisting essentially of sulphur, and rubber.

2. Insulating material for linings and other uses, comprising granulated cork, a binder consisting essentially of sulphur, and latex.

3. A process for the manufacture of an agglomerate comprising granulated cork and sulphur as the essential binder for the cork granules, which comprises heating the cork granules to a temperature sufficient to melt the sulphur, and spraying the sulphur in the form of powder on the heated granules, thereby to cause the sulphur to melt and adhere to the granules and the granules to adhere to each other.

4. A process for the manufacture of an agglomerate comprising granulated cork and sulphur as the essential binder for the cork granules, which comprises pouring molten sulphur on a body of the loose cork granules while stirring the mass.

PIERRE MICHEL JUSTIN BARDOU-JOB.  
HENRI FRANCIS HÉBRARD.